

# United States Patent [19]

Eriksson et al.

[11] 3,867,136

[45] Feb. 18, 1975

[54] DECARBURISATION OF CHROMIUM CONTAINING IRON, COBALT OR NICKEL BASED ALLOYS

[75] Inventors: Lars Anders Eriksson; Karl-Erik Oberg, both of Hagfors, Sweden

[73] Assignee: Uddeholms Aktiebolag, Hagfors, Sweden

[22] Filed: Oct. 5, 1973

[21] Appl. No.: 403,854

[30] Foreign Application Priority Data

Oct. 6, 1972 Sweden..... 12907/72

[52] U.S. Cl..... 75/60, 75/59, 75/82

[51] Int. Cl..... C21c 5/32

[58] Field of Search..... 75/59, 60, 82

[56] References Cited

UNITED STATES PATENTS

2,855,293 10/1958 Savaro..... 75/60

3,706,549 12/1972 Knuppel..... 75/60

FOREIGN PATENTS OR APPLICATIONS

1,450,718 7/1966 France..... 75/60

Primary Examiner—L. Dewayne Rutledge

Assistant Examiner—Peter D. Rosenberg

Attorney, Agent, or Firm—Cushman, Darby & Cushman

[57]

ABSTRACT

In a process for decarburising stainless steel by blowing the molten steel with a mixture of oxygen together with steam and/or ammonia, blockage of gas inlet is avoided by passing the mixture of oxygen together with steam and/or ammonia through the inner section of a tuyere comprising at least two coaxial pipes and passing through the outermost section of the tuyere a gas e.g. oxygen and steam or oxygen and nitrogen, which undergoes an exothermal reaction when it contacts the molten alloy.

11 Claims, 1 Drawing Figure

PATENTED FEB 18 1975

3,867,136



DECARBURISATION OF CHROMIUM  
CONTAINING IRON, COBALT OR NICKEL BASED  
ALLOYS

The present invention relates to an improved process for reducing the carbon content of an iron, cobalt or nickel based alloy containing carbon and at least 10 percent chromium, particularly stainless steels, by introducing into the molten alloy, oxygen together with steam and/or ammonia which decompose in the melt yielding hydrogen. This hydrogen is able to influence the partial pressure of carbon monoxide (derived by oxidation of the carbon) in the melt and so control the extent of oxidation of chromium and other readily oxidisable components in the melt during the decarburisation.

The basic decarburisation process is described in detail in U.S. Pat. application Ser. No. 295355 filed Oct. 10th 1972 by M. K. O. Johnsson and L. A. Ericksson. Briefly, this decarburisation process involves the use of a mixture of oxygen with a high percentage of steam and/or ammonia. During the main part of the decarburisation period the volume ratio oxygen: steam + ammonia should preferably be less than 3 : 1 and a recommended value is between 1 : 1 and 1 : 10. This high content of steam and/or ammonia has a great cooling effect on the steel, the more so since the gas mixture should be injected at a speed which exceeds that of sound. As a result the tuyeres show a marked tendency to get blocked by solidification of the melt. The present invention provides a method of decarburisation in accordance with the general procedure of the above described Patent Application but under conditions which reduce the tendency for the tuyeres to get blocked without giving rise, simultaneously, to new problems due to excessive energy development in the tuyere area, which would entail an unacceptable rate of wear of the tuyeres and/or of the area in the proximity of these.

The present invention provides a method of reducing the carbon content of an iron, cobalt or nickel based alloy containing carbon and at least 10 percent by weight chromium by introducing into the molten alloy oxygen and a hydrogen yielding gas which is steam or ammonia or mixtures thereof wherein a mixture of oxygen and the hydrogen yielding gas is introduced into the molten alloy through an inner section of a tuyere comprising at least two coaxial pipes, the amount of hydrogen yielding gas being sufficient to bring about an endothermal reaction when the hydrogen yielding gas meets the molten alloy, and introducing through the outermost section of the tuyere a gas which undergoes an exothermal reaction when it meets the molten alloy.

The invention will now be described more in detail, with reference to the accompanying drawing, which shows the principles for the design of a tuyere for use in the invention.

In the figure, tuyere 1 consists of two concentric pipes, an inner pipe 2 and an outer pipe 3. The pipes can, for example, be made of copper, carbon steel or stainless steel. The opening between the pipes is indicated by 4. Speed, flow and number of tuyeres will determine the size of the tuyeres. A suitable diameter for the inner pipe is 5 to 15 mm. and the width of opening 4 should be at least 0.5 mm but not more than 2 mm. Tuyere 1 extends through the bottom 6 (or the wall) of the converter or other process vessel, containing the

melt 5 in process of decarburization. Tuyere 1 has a contraction 7, which divides the tuyere into two parts, namely a forward part 8 and a rear part 9. Forward part 8 has a narrower cross-section than rear part 9, but the ratio of the cross sectional areas of each of these two parts is equal. This arrangement brings about a pressure reduction in the delivery lines when the tuyere has undergone wear reaching the area of the contraction. This lowered pressure can be used as an indication that the tuyere or the bottom of the converter needs replacing. In an embodiment of the invention aiming at exploiting this facility, the lines connected to the tuyere are therefore connected to suitable regulating members, which sense and register the pressure in the lines.

In order to ensure sufficient impulse when the gas mixture is injected into the melt, the injection speed should exceed the critical speed, i.e., that of sound. The total flow of gas through the tuyere or the tuyeres should be 0.5 to 5 standard cubic metres per metric ton of melt per minute (St.m<sup>3</sup>/ton/min). Preferably 0.5 to 3 St.m<sup>3</sup>/ton/min.

In implementing the method according to the invention the mixture of oxygen with steam and/or ammonia is injected through the inner pipe 2. The steam and/or ammonia content of the mixture should be at least 25 percent by volume, and in practice is usually 50 to 90 percent by volume (volume ratio oxygen : steam and/or ammonia 1 : 1 - 1 : 10). Under these circumstances, the gas mixture used for the decarburisation has a strong cooling effect because of the large amount of thermal energy required for the decomposition of the steam and/or ammonia. In order to reduce the tendency for the tuyere to become blocked by solidification of the melt, a gas mixture having an exothermal reaction with the melt in the area of the orifice of the tuyere is injected through opening 4 between inner pipe 2 and the outer pipe 3. The "exothermal" gas will normally contain a large proportion of oxygen but the proportion of oxygen should not be so high as to cause damage to the tuyere itself or to the parts adjacent to it as a result of excessive heat generation close to the tuyere orifice. Examples of suitable gas mixtures to be injected through opening 4 are

1. 40 - 80% O<sub>2</sub> : 60-20% steam
2. 10 - 50% O<sub>2</sub> : 90-50% argon
3. 5 - 30% O<sub>2</sub> : 95-70% N<sub>2</sub>, all percentages being by volume.

Combinations of these gas mixtures are also possible. The rate of flow through opening 4, preferably amounts to less than 20 percent, and particularly 10-15 percent of total volume of gas flow through the tuyere.

The tuyere described above contains only two concentric pipes but it is possible to operate in accordance with the invention using a tuyere having 3 or more concentric pipes. In this case, the "endothermic" gas mixture is injected through one or more inner sections of the tuyere but not through the outermost section while the "exothermal" gas mixture is injected through the outermost section. This arrangement is also convenient when it is desired to inject ammonia separately from oxygen in which case oxygen is injected through one inner section, ammonia is injected through a different inner section and the "exothermal" gas mixture is injected through the outermost section.

In the drawing, only one tuyere is shown but in practice, the decarburisation will be carried out using several tuyeres of this type.

The type of alloys which can be treated in this invention and the general details of the decarburisation and ancillary refining steps used in this invention are the same as those disclosed in the patent application mentioned in the second paragraph of this specification and those disclosures are incorporated in this specification by this reference.

We claim:

1. A method of reducing the carbon content of an iron, cobalt or nickel based alloy containing carbon and at least 10 percent by weight chromium by introducing into the molten alloy oxygen and at least one hydrogen yielding gas selected from the group consisting of steam and ammonia wherein a first mixture consisting essentially of a minor proportion by volume of oxygen and a major proportion by volume of the hydrogen yielding gas is introduced into the molten alloy through an inner section of a tuyere comprising at least two coaxial pipes and having at least one inner section and an outermost section, the amount of hydrogen yielding gas being sufficient to bring about an endothermal reaction when the hydrogen yielding gas meets the molten alloy, and introducing through the outermost section of the tuyere a second mixture which is a gas which undergoes an exothermal reaction when it meets the molten alloy and which second mixture consists essentially of oxygen and a cooling gas.

2. A method according to claim 1 where the volume of gas flowing through the outermost section of the tuyere is not more than 20 percent of the total volume of gas flowing through the tuyere.

3. A method according to claim 2 where the flow through the outermost section is 10 - 15 percent by volume of the total flow.

4. A method according to claim 1 wherein the gas flowing through the outermost section contains 40 - 80 percent by volume oxygen and 60 - 20 percent by volume steam.

5. A method according to claim 1 wherein the gas flowing through the outermost section contains 5 - 30 percent by volume oxygen and 95 - 70 percent by volume nitrogen.

10. A method according to claim 1 wherein the gas flowing through the outermost section contains a major amount by volume of nitrogen and minor amounts by volume of oxygen and steam.

15. A method according to claim 1 wherein at least one tuyere has a contraction in its cross sectional area at a position spaced apart from that end of the tuyere opening into the melt and at least one feed line to the tuyere is provided with a pressure sensing device which can indicate, by recording pressure variation in the feed line, when the tuyere has been corroded away as far as the contraction.

20. A method according to claim 1 wherein the alloy is a stainless steel.

25. A method according to claim 1 wherein the volume ratio of oxygen to steam and/or ammonia in the gas mixture introduced through the inner section of the tuyere is 1 : 1 to 1 : 10.

30. A method according to claim 1 wherein the rate of flow of the gases introduced into the molten alloy is 6.5 - 5 standard cubic metres per metric ton per minute.

35. A method according to claim 1 wherein the cooling gas is at least one selected from the group consisting of steam, nitrogen and argon.

\* \* \* \* \*